

Oct. 18, 1960

H. L. BROWNBACk

2,956,908

OIL RESISTANT COATED GASKET MATERIAL

Filed April 25, 1956



INVENTOR.  
HENRY L. BROWNBACk

BY  
*Edward Thomas*

ATTORNEY



the material of the present invention is sprayed thereon before the surfaces are brought together.

It has also been found possible to apply the mixture carrying a suitable thinner by a roller type applying device. For this purpose a less volatile thinner, such as di-ethylene glycol, may be more satisfactory. Such a procedure works because the material of the present invention remains tacky instead of becoming hard as the thinner evaporates.

That thinner is removable by infra red lamps as it passes through a tunnel.

One of the problems involved in the building of automobile engines has been the problem of providing tight joints where a cover plate or other separate part is united to the body of the engine because a gasket to work satisfactorily in such a joint has to be resistant to high temperatures, to gasoline, to oils and must yet not become brittle in the mold as when the engine is left standing for a long time exposed to the winter weather.

While many blown oils may be satisfactory for some purposes, the best seems to be a blown castor oil product as described below. Such an oil has a characteristic tackiness which is found a suitable test for other blown oils when analogous compositions are produced for other utilities.

In the accompanying drawing is shown a device found suitable for producing the most satisfactory blown oil for incorporating into the present invention. In that drawing

Fig. 1 is a diagrammatic sectional side view of the blowing apparatus.

Fig. 2 is an enlarged sectional view on the line 2—2 of Fig. 1.

Fig. 3 is a similar view on the line 3—3 of Fig. 1.

The device shown includes not only the container and means for blowing the oil, but also shows a viscometer embodied therein.

In the form shown a mixture of 120 liters of raw castor oil with 130 liters of castor oil blown to a viscosity of 30 centipoises, as measured on a standard viscosity measuring machine, is placed in the container 10 having a height from bottom to inside of cover rim 11 about 900 millimeters and a radius of about 750 millimeters, and air is blown in at a temperature of 205° C. on a volume of 90 cubic meters per hour at a pressure of 1.4 kilograms per square centimeter at the entrance to the kettle.

The oil fills the kettle to a height of about 670 millimeters and the air enters through a vertical pipe 12 extending down to an annular distributor passage 13 clearing the bottom by about 100 millimeters.

From this manifold or distributor 13 extend radially six equally spaced round distribution pipes 14 about 20 millimeters internal diameter and perforated around their bottom holes with closely set 2 millimeter openings 15 to the air is directed principally downward.

The pipes 14 terminate about 50 millimeters clear of the inside of the wall of the container 10, thus allowing oil to circulate freely around them.

The oil is agitated during the admission of air by a four-bladed variable pitch agitator 16 turning at about 1200 to 1500 r.p.m. carried at the bottom of a vertical power driven shaft 17 so that the blades, about 340 millimeters from tip to tip keep the oil circulating through the open center of the manifold 13, and clear the tie rods 18 which support the manifold 13 near the periphery.

The best results, predictably uniform, were obtained by the procedures described below.

The oil after being placed in the container 10 was

"blown" by entering air through the pipes 14 and agitated by the agitator at about 1200 r.p.m. until the oil reaches a temperature of 205° C., usually about 45 minutes, as shown on the thermometer 19 with its bulb immersed in the oil, the oil is tested by being drawn in through the submerged nozzle 20 of a viscometer 21.

This viscometer takes the form of a 20 millimeter long tube 22 fixed in the top of the container 10 and carrying the nozzle 20 with a central cylindrical opening 23 three millimeters in diameter, spreading to eight millimeters in twelve millimeters and opening into the tube 22 at the end of 20 millimeters more.

The tube 22 terminates at the top in a glass bulb 24 holding one liter between its index lines, and the bulb 24 is connected by a passage 25 to a three way cock 26 turnable to open it to a suction line 27, or to a line 28 open into the top of the container 10.

When the blown oil has reached the temperature of 205° C. and the suction is turned on the tube 22, the oil fills the bulb 24 in about 55 to 58 seconds, the impeller being stopped but blowing air continued.

The bulb 24 is then emptied back into the container 10 by turning the cock 26 and the blowing continued until the desired oxidized consistency is reached, usually four to four and one-half hours, and the consistency is measured to this end by measuring the time to refill the bulb 24, which should be 80 to 82 seconds.

It should be noted that the oil gives off acrid vapors and other volatiles while being blown and these are carried off by a large vent 29, and may be absorbed by sulfuric acid, preferably carried in broken earthenware through which the gases bubble.

After the 82 second reading is reached the impeller is stopped but air is blown in until the temperature has dropped to 100° C. to 110° C. Then anti-oxidant is added (melted, if need be), any solvent used is added also any other additives, such as fillers.

It is found that workers in this process soon learn to empirically test an oil by observing its tackiness and many blown oils they thus test and approve are at least fairly satisfactory for the present invention to replace the castor oil thus blown.

Having thus described certain embodiments of the invention, what is claimed is:

45 Gasket material having on its outer surface a coating of an adherent sealing composition prepared by combining a blown castor oil forming a tacky gel and having a viscosity of at least 2,000 poises with a dimethyl silicone having a viscosity of at least 30,000 centistokes in 50 the proportion of approximately 9 to 1 by weight.

#### References Cited in the file of this patent

#### UNITED STATES PATENTS

|    |           |                |                |
|----|-----------|----------------|----------------|
| 55 | 2,054,801 | Bailey         | Sept. 22, 1936 |
|    | 2,129,281 | Lincoln et al. | Sept. 6, 1938  |
|    | 2,317,487 | Schuelke       | Apr. 27, 1943  |
|    | 2,327,450 | Parker         | Aug. 24, 1943  |
|    | 2,442,196 | Coggeshall     | May 25, 1948   |
| 60 | 2,466,642 | Larsen         | Apr. 5, 1949   |
|    | 2,467,178 | Zimmer et al.  | Apr. 12, 1949  |
|    | 2,491,843 | Wilcock        | Dec. 20, 1949  |
|    | 2,523,065 | Sage           | Sept. 19, 1950 |
|    | 2,557,928 | Atkinson       | June 26, 1951  |
| 65 | 2,635,060 | Cheronis       | Apr. 14, 1953  |

#### OTHER REFERENCES

McGregor: "Silicones and Their Uses," McGraw-Hill, 1954, pp. 176-177, 201, 207, 217 relies on.